

Jan. 17, 1950

D. R. HOOD ET AL

2,495,063

HEAT TREATMENT OF COPPER-NICKEL-MANGANESE ALLOYS

Filed Aug. 2, 1945

4 Sheets-Sheet 1



INVENTORS

Donald R. Hood  
Stanley R. Hood  
Barnes, Kisselle, Laughlin, Leisick

ATTORNEYS.

Jan. 17, 1950

D. R. HOOD ET AL

2,495,063

HEAT TREATMENT OF COPPER-NICKEL-MANGANESE ALLOYS

Filed Aug. 2, 1945

4 Sheets-Sheet 2

FIG. 2.



INVENTORS.

Donald R. Hood  
BY Stanley R. Hood  
Garnes, Kisselle, Laughlin & Powers

ATTORNEYS.

Jan. 17, 1950

D. R. HOOD ET AL

2,495,063

HEAT TREATMENT OF COPPER-NICKEL-MANGANESE ALLOYS

Filed Aug. 2, 1945

4 Sheets-Sheet 3



BY

Donald R. Hood  
Stanley R. Hood  
Barney Kinsella, Laughlin & Frazer

ATTORNEYS.

INVENTORS.  
Donald R. Hood  
Stanley R. Hood  
Barney Kinsella, Laughlin & Frazer

Jan. 17, 1950

D. R. HOOD ET AL

2,495,063

HEAT TREATMENT OF COPPER-NICKEL-MANGANESE ALLOYS

Filed Aug. 2, 1945

4 Sheets-Sheet 4

FIG. 5.



Effect of Time at solution temperature on time-hardness curve. Curve shows average values & variations for 1/2, 1, 2, & 4 hours at 1100°F. Water quenched samples.



FIG. 6.

INVENTORS.  
Donald R. Hood  
Stanley P. Hood  
BY Barnes, Kegelle, Laughlin  
"Faisel" ATTORNEYS.

## UNITED STATES PATENT OFFICE

2,495,063

## HEAT-TREATMENT OF COPPER-NICKEL-MANGANESE ALLOYS

Donald R. Hood and Stanley R. Hood, Detroit, Mich., assignors, by mesne assignments, to Chicago Development Company, Chicago, Ill., a corporation of Illinois

Application August 2, 1945, Serial No. 608,440

6 Claims. (Cl. 148—12.7)

1

This invention relates to improvements in heat treating procedure for copper-nickel-manganese alloys such as are described in Patents No. 2,234,552 and No. 2,270,868. The alloys of these patents, which seem to be of most commercial importance at the present time contain 50-75% copper, with the remainder substantially equal parts of nickel and manganese. We have found by modifying temperatures and rates of temperature change, heat-treated alloys can be made with improved physical properties, which require less time for developing hardness and do not require an objectionable, high solution temperature treatment preliminary to hardening.

Patent No. 2,234,552, referred to above, specifies quenching the alloys from 900° C. or higher and states further that if a lower quenching temperature is used, "the final hardening or aging step will be less effective." Such a statement can be made in reference to precipitation hardening alloys generally, that is, there is a certain minimum temperature from which quenching must take place to maintain a supersaturated solution from which a constituent may subsequently be precipitated by heating the alloy below the quenching temperature. We have found not only does such a procedure not apply to these alloys, but, in fact, the opposite is true, namely, the farther below 900° C. quenching takes place, the more effective the aging treatment. The only limit in decreasing the quenching temperature is the overlapping of the aging temperature range.

Even further removed from the usual precipitation hardening procedure is the insensitivity of these alloys to rate of cooling from the quenching temperature. Ordinarily it is necessary to cool rapidly from the solution temperature to maintain a high solubility of the precipitate in the alloy. We have found these alloys to harden through an entirely different mechanism. The alloys may be water quenched, air cooled, or even furnace cooled without appreciably changing either the maximum hardness which may be produced or the time required for aging.

That such an insensitivity to cooling rate is not due to mere sluggishness of the alloy, but to a different hardening mechanism is shown by its "reversible" heat treatment. We have found that 5 hardening and softening can be alternately produced by temperature changes without the intermediate quenching or solution step.

In the drawings:

Fig. 1 shows the range over which the copper-nickel-manganese alloys of our invention are hardenable. In Figs. 2 to 6 the graphs relate to an alloy containing 60% copper, 20% nickel, and 20% manganese. It will be noted that Fig. 1 corresponds to Fig. 1 of Patent No. 2,234,552 and, as in said patent, the shaded or cross-hatched area represents the hardenable range of the alloys. The dotted area represents alloys which are hard as cast, are not easily fabricated, and do not fall 15 within the scope of the present invention. The line MnNi substantially bisects the shaded area and corresponds with the hypothetical compound MnNi.

Fig. 2 shows the effect of solution temperature 20 on the hardenability of such alloy.

Fig. 3 shows the effect of time at solution temperature on the hardness of such alloy.

Fig. 4 shows the effect of solution temperature 25 on the time hardness curve.

Fig. 5 shows the time hardness curve for such alloy.

Fig. 6 shows the effect of time at solution temperature on the time hardness curve for such 30 alloy.

Fig. 2 shows the effect of solution temperature 35 on the hardenability of an alloy containing 60% copper, 20% nickel, 20% manganese. Samples were aged at 750° F. for periods of time up to fifty-six hours. This is ample time for most of the aging to take place in all samples. The hardness, grain size, and tensile properties are tabulated for fully hardened samples having various solution temperatures as follows:

| Annealing Temp., °F. | Proportional Limit, 0.1 Offset | .1% Yield Stress | .2% Yield Stress | Tensile Strength | Young's Modulus | Elongation, Percent | Hardness |
|----------------------|--------------------------------|------------------|------------------|------------------|-----------------|---------------------|----------|
| 1,100                | 140,150                        | 184,350          | —                | 230,100          | 21.29           | 1.9                 | 429      |
| 1,650                | 71,950                         | 81,400           | 85,000           | 107,300          | 22.53           | 14.4                | 224      |
| 1,650                | 76,650                         | 87,850           | 91,000           | 109,400          | 22.95           | 14.8                | 224      |
| 1,800                | 64,100                         | 75,400           | 75,800           | 89,700           | 19.57           | 11.8                | 215      |
| 1,800                | 66,100                         | 70,150           | 73,000           | 88,600           | 19.44           | 14.8                | 215      |

Photomicrographs show the grain size for the 1800° F. annealed material to be approximately ten times the size of the 1650° F. anneal and more than one thousand times larger than the 1100° F. material.

The high solution temperatures produce very large grain sizes, low hardness, and comparatively poor tensile values.

Fig. 2 also shows time-hardness curves for the same three samples. It will be noted that not only is the hardness increase less pronounced for the samples having high solution temperatures, but the rate of hardening is much slower. Fig. 3 shows the drop in hardness of cold rolled samples after being heated to 950, 1000, 1050, and 1100° F. for time intervals of  $\frac{1}{2}$ , 1, 2 and 4 hours. It is shown that 1000, 1050, or 1100° F. may be used with approximately the same drop in hardness resulting. At 1100° F. full softening takes place in less than  $\frac{1}{2}$  hour. At 1050° F. slightly longer heating is required, and at 1000° F. over one hour at temperature is required. At 950° F. a remarkable phenomenon occurs in that both softening and hardening occur at the same temperature. At this temperature the hardness first drops, probably due to relief of cold work stress, and then as the metal remains at this temperature, aging begins and the hardness increases. This makes it possible to give a stress relieving heat treatment prior to the aging treatment. Such a treatment greatly decreases distortion during aging. This has been verified by actual tests on production parts. The material can be stress relieved either by heating the metal in a continuous strip or strand annealing furnace, or blanked elements may be stress relieved before the final forming and aging operations. This stress relieving step does not appreciably affect either the subsequent hardening rate or the physical properties as compared to rolled and aged material.

Probably the most useful characteristic of the heat treatment of these alloys is the discovery of their "reversible" hardening. Generally, precipitation hardening alloys harden most rapidly by using as high an aging temperature as possible. If, however, the temperature used is too high, resolution of the precipitate occurs, and it is not possible to obtain full hardening without repeating the quenching treatment and reaging at a lower temperature. We have found the copper-nickel-manganese alloys to follow an entirely different heat treating pattern. These alloys have most rapid hardening and obtain maximum hardness at an intermediate aging temperature. Using a higher temperature increases, rather than decreases, the hardening time. If, however, a fully hardened sample is reheated above the optimum aging temperature, the hardness is "drawn" to a lower value, depending on the "drawing" temperature. By selecting the temperature correctly a fully hardened sample can be drawn to any hardness between full hard and dead soft. Within practical limits this drawing depends only on temperature and not on time. The time at temperature may vary between one-half hour and two hours without affecting the hardness drop appreciably. The unique feature of this "drawing," however, is that full hardness may again be developed by merely heating to the normal aging temperature. Fig. 4 shows the temperature-hardness relation in drawing 60% manganese, 20% copper, 20% nickel alloy. It will be noted that for annealing temperatures of 1000, 1050, or 1100° F. the hard-

nesses are substantially identical after ten hours of aging. It is interesting to note that even the slight differences in annealing temperatures in the range 1000-1100° F. show corresponding differences in hardening rates, that is, in the first six hours most rapid hardening occurs when the lowest possible annealing temperature is used. Although the grain size for samples annealed at 1000, 1050, and 1100 degrees is all very fine, there is a measurable difference—the finest grain, of course, occurring at the 1000 degree anneal.

Fig. 5 shows the time-hardness curve for a sample of this alloy. Instead of reaching a peak hardness and then softening on further heating at the same temperature, this alloy shows no hardness drop after thirty days at the optimum aging temperature. The hardening effect is cumulative, that is, the hardening which occurs in a ten hour period is exactly the same as that which would build up in ten separate cycles of one hour each. From these characteristics it is possible to make heat treated elements with a minimum of variation in hardness. Any part which is not as hard as required can be reheated to the aging temperature for additional hardening. Any element which is harder than specified can be "drawn" back to the correct hardness. If elements already hardened require a change in form or machining as a result of change in design, it is only necessary to heat to slightly above the aging temperature to soften the material and after making the necessary alterations, reheat at the aging temperature to reharden. Local areas of hardened parts may be softened if desired.

As already stated, quenching in the ordinary sense of the word is not required as a prerequisite to hardening. The alloys may be furnace cooled and still age as well as a sample quenched from the same temperature. If cooling in the furnace takes place very slowly, partial hardening will occur as the metal passes through the aging temperature range. Therefore, the alloys can be hardened by iso-thermal heating, that is, merely dropping from the solution temperature to the aging temperature and holding at the latter until the desired amount of aging is accomplished. The commercial application of such a treatment is in the silver soldering of these alloys. Parts to be silver brazed may be run through a two zone continuous furnace in which brazing occurs in the first at a temperature which melts the solder, and aging takes place in the second which operates at the aging temperature.

In the treatment of copper-nickel-manganese alloys outlined above, one starts with a cast alloy which has had its grain size substantially reduced by conventional methods such, for example, as both hot and cold working or rolling, hot working or rolling from about 1650° F. down to room temperature or down to solution temperature and also cold working plus annealing. Hot rolling is used primarily to reduce the size of the casting or ingot and also refines the cast grain some. Cold rolling elongates the grains and develops slip planes. The best physical properties are obtained when the alloy is subjected to cold rolling subsequent to annealing and before age hardening. The annealing step relieves strains and reorientates the grain structure so that the alloy is softer. If the part being fabricated permits, it is possible to cold roll the alloy after annealing and before age hardening.

For the alloys falling within the shaded area

of Fig. 1, the annealing temperature range is from about 975° F. to about 1300° F. with an annealing temperature of 1050° F. preferred for the alloy comprising essentially 60% copper, 20% manganese, 20% nickel by weight. The hardening temperature range for the alloy comprising 60% copper, 20% manganese, 20% nickel, or lesser amounts of manganese and nickel, is from about 500° F. to about 800° F. with a hardening temperature of 750° F. preferred. Where the manganese and nickel each exceeds 20%, the hardening temperature range is from about 500° F. to about 950° F. Where the manganese and nickel each exceeds 20% of the alloy or more than 40% together of the alloy by weight, the upper limit of the hardening temperature range is higher than for the alloy comprising essentially 60% copper, 20% manganese, 20% nickel. If the manganese and nickel each exceeds 20% of the alloy, or together exceeds 40% of the alloy, the higher temperatures in the above set forth annealing temperature range are preferably used. For example, an alloy comprising 40% copper, 30% manganese and 30% nickel should be annealed at about 1250° F. By annealing and hardening within the temperature ranges above set forth, an alloy having even better physical properties than those disclosed in the above said Dean patent can be obtained with substantially less cold rolling after annealing and before age hardening. In fact, with our annealing and hardening steps we can obtain a hardened alloy having better physical properties than those obtained by the treatment outlined in the Dean patent with only a 30% reduction in size of the ingot or casting by cold rolling between annealing and age hardening as contrasted with a 70% reduction in size by cold rolling between quenching and aging when Dean's quenching and aging procedure is followed.

We claim:

1. The improvement in hardening copper-manganese-nickel alloys falling within the shaded area of Figure 1, which consists in working the alloy to reduce its grain size, then heating it to a temperature between 975° F. and 1300° F. to fully soften the alloy, cooling the alloy at a rate greater than that obtaining in ordinary furnace cooling and then heating the alloy to a temperature of 500° F. and 950° F. for a period of at least 10 hours whereby to obtain a hardened alloy with improved properties.

2. The method of claim 1 further characterized by cold working the alloy before heating to 500° F. to 950° F. to harden it.

3. The improvement in the method of treating copper-manganese-nickel alloys, having 60% copper, 20% manganese and 20% nickel within the usual commercial composition limits for such alloys, which consists in the working of the alloy to reduce its grain size, heating to a temperature of about 1050° F. for a period of at least 30 minutes to fully soften the alloy, cooling the alloy at a rate greater than that obtaining in ordinary furnace cooling and then heating the alloy to a temperature of about 750° F. for not less than 10 hours whereby to harden the alloy and improve the ductility of such hardened alloy.

4. The method of claim 3 further characterized by cold working the alloy before heating to about 750° F. to harden the alloy.

5. The method of treating an alloy hardened according to claim 1 to partially soften then fully reharden it, which consists in the steps of heating to a temperature of 975° F. to 1300° F. for a period insufficient to fully soften the alloy and then heating the alloy to a temperature of 500° F. to 950° F. for a period of at least 10 hours.

6. The method of claim 5 further characterized by cold working the partially softened alloy before heating it to reharden it.

DONALD R. HOOD.  
STANLEY R. HOOD.

#### REFERENCES CITED

The following references are of record in the 35 file of this patent:

#### UNITED STATES PATENTS

| Number    | Name        | Date          |
|-----------|-------------|---------------|
| 1,816,509 | Wise        | July 28, 1931 |
| 2,201,555 | Corson      | May 21, 1940  |
| 2,234,552 | Dean et al. | Mar. 11, 1941 |

#### OTHER REFERENCES

- "Practical Metallurgy," Sachs and Van Horn, 45 1940, American Society for Metals, Cleveland, Ohio, pp. 123 and 124.  
 "Age Hardening of Metals," 1940, American Society for Metals, Cleveland, Ohio, pp. 60, 61.  
 "Transactions," vol. 34, 1945, American Society 50 for Metals, Cleveland, Ohio, pp. 481-504.